

# UNITED STATES PATENT OFFICE.

WALTER RUNGE, OF CHESTER, PENNSYLVANIA, ASSIGNOR TO E. I. DU PONT DE NEMOURS POWDER COMPANY, OF WILMINGTON, DELAWARE, A CORPORATION OF NEW JERSEY.

## COMPOSITION FOR DETONATING EXPLOSIVE CHARGES.

1,168,746.

Specification of Letters Patent. Patented Jan. 18, 1916.

No Drawing.

Application filed June 12, 1913. Serial No. 773,199.

*To all whom it may concern:*

Be it known that I, WALTER RUNGE, of Chester, in the county of Delaware, and in the State of Pennsylvania, have invented a certain new and useful Improvement in Compositions for Detonating Explosive Charges, and do hereby declare that the following is a full, clear, and exact description thereof.

10 My invention relates particularly to an improvement in compositions used for detonating explosive charges, such for example as charges of dynamite.

Hitherto detonators of this character have 15 usually contained fulminate of mercury, either throughout the whole charge in the detonator, or in the priming charge merely, where the detonator contains a main charge which cannot be detonated by a fuse and a 20 priming charge to be detonated by a fuse. Such detonator compositions have usually been made by mixing with the fulminate of mercury a quantity of an oxidizing agent, such for example as chlorate of potassium. 25 Certain other explosives have been substituted for the fulminate of mercury, such for example as lead azid  $Pb(N_3)_2$ , diazo compounds, etc. Such primary detonators do not 30 themselves contain sufficient oxygen for complete combustion, and it has therefore generally been thought necessary to add an oxidizing agent, such for example as chlorate of potassium. I have, however, discovered that a more effective detonation can be obtained 35 by using instead of an oxidizing agent a nitro-hydrocarbon of the aromatic series, such for example as trinitrotoluene.

While my invention is capable of being carried out in many different ways, for the 40 purpose of illustration I may produce a detonating composition in accordance with my invention in the following manner:

Such a detonating composition may be made by adding to 90 parts of fulminate of 45 mercury 10 parts of trinitrotoluene. Or a composition may be formed by adding to 70 to 95 parts of lead azid, 5 to 30 parts of trinitrotoluene. For example, a particular composition may be made by adding to 80 50 parts of lead azid 20 parts of trinitrotoluene.

The composition containing lead azid, and having the proportions referred to, forms an exceedingly good detonating compound and gives excellent results when used as a priming charge for detonators containing a main 55 charge of trinitrotoluene, picric acid, etc., although it also gives excellent results with other similar explosives. The lead azid composition may be readily ignited by a fuse and detonates with such a high velocity that 60 a small amount of this mixture is sufficient to completely detonate the main charge. There is no difficulty in producing the mixture of the ingredients. If desired, the constituents may be mixed with a small amount 65 of binding material, such as gum arabic. The amount of gum arabic used in the above compositions is preferably from 0.01 to 0.1 parts. To this purpose 0.02 parts of gum arabic may be added, for example, to the 70 composition containing 80 parts of lead azid and 20 parts of trinitrotoluene. The mixture so obtained is fine grained and free running, and can be readily loaded into a detonator shell. The pressing of the charge 75 may be accomplished in the usual manner. Such a composition is suitable for use either as the entire charge of a detonator or merely as a priming charge therein, as it will detonate a main charge of less sensitive material, 80 very effectively.

While I have described my invention above in detail, I wish it to be understood that many changes may be made therein without departing from the spirit of my invention, and that the terms used therein shall be interpreted in their broad significance. For example, the word detonator is to be understood as including among other devices dynamite caps which are to be ignited 85 by a flame from a fuse, as well as electric detonators in which the charge is ignited by an electric current.

I claim:

1. A charge for blasting caps containing 95 a mixture of 70 to 95 parts of lead azid and 5 to 30 parts of trinitrotoluene.
2. A priming charge for blasting caps containing a mixture of 70 to 95 parts of lead azid and 5 to 30 parts of trinitrotoluene. 100

3. A charge for blasting caps containing a mixture of 80 parts of lead azid and 20 parts of trinitrotoluene.

4. A priming charge for blasting caps containing a mixture of 80 parts of lead azid and 20 parts of trinitrotoluene.

In testimony that I claim the foregoing I have hereunto set my hand.

WALTER RUNGE.

Witnesses:

CHAS. G. WORRILLOW,  
WM. P. LEAR.